

[54] SYNERGISTIC MIXTURE OF ADIAMINE AND ALKALIMETALAMIDE AS AN ANTIOXIDANT COMPOSITION AND LUBRICANTS CONTAINING SAME

[75] Inventors: Michael Gavin Bird, Weybridge; Keith Aled Wyn Parry, Camberley, both of England

[73] Assignee: The British Petroleum Company Limited, London, England

[22] Filed: Jan. 5, 1972

[21] Appl. No.: 215,646

[30] Foreign Application Priority Data

|               |                     |          |
|---------------|---------------------|----------|
| Jan. 18, 1971 | United Kingdom..... | 2350/71  |
| Aug. 12, 1971 | United Kingdom..... | 37868/71 |
| Sept. 7, 1971 | United Kingdom..... | 41589/71 |

[52] U.S. Cl..... 252/49.7; 252/50; 252/400 R; 252/401

[51] Int. Cl..... C10n 1/10

[58] Field of Search..... 252/49.7, 50, 400 R, 401

[56] References Cited

UNITED STATES PATENTS

|           |        |                       |          |
|-----------|--------|-----------------------|----------|
| 3,247,111 | 4/1966 | Oberright et al. .... | 252/50 X |
|-----------|--------|-----------------------|----------|

FOREIGN PATENTS OR APPLICATIONS

|           |         |                     |          |
|-----------|---------|---------------------|----------|
| 1,047,278 | 11/1966 | United Kingdom..... | 252/50   |
| 655,985   | 1/1963  | Canada.....         | 252/49.7 |

OTHER PUBLICATIONS

Houben-Weyl, "Methoden der Organischen Chemie," Vol. 10/2, pgs. 754-755 (1967).

Migrdichian, "Organic Synthesis," Vol. II, pg. 1452 (1957).

Musso, "Chemical Abstracts," Vol. 54, page 5659, titled "The Decomposition Products of Tetraphenylhydrazines" (1960).

Primary Examiner—Patrick P. Garvin

Assistant Examiner—Andrew H. Metz

Attorney, Agent, or Firm—Morgan, Finnegan, Durham & Pine

[57] ABSTRACT

Antioxidant composition comprises a synergistic mixture of a diamine, e.g. N,N,N'-tris-(4-t-octylphenyl)-4-t-octyl-1,2-phenylene diamine, di-DODPA, and an alkali metal derivative of the same or similar diamine. The composition is particularly suitable for use in synthetic ester lubricants.

14 Claims, No Drawings

**SYNERGISTIC MIXTURE OF ADIAMINE AND  
ALKALIMETALAMIDE AS AN ANTIOXIDANT  
COMPOSITION AND LUBRICANTS CONTAINING  
SAME**

This invention relates to high temperature antioxidants and to lubricants containing them, particularly synthetic lubricants suitable for use under the severe high temperature conditions that exist in the operation of modern aero gas turbine engines.

The problem of thermal stability in aero gas turbine lubricants can be satisfactorily handled by the use of certain hindered ester basestocks which generally also have good low temperature properties, being fluid in many cases at temperatures of  $-40^{\circ}$  or below. A more difficult problem that has to be faced however, is the problem of oxidation stability and resistance to corrosion which arises owing to the fact that the lubricants have to operate at high bulk oil temperatures (about  $200^{\circ}\text{C}$ ) in contact with air. These conditions have the effect of greatly accelerating the oxidative deterioration of the lubricant which generally results in an increase in its viscosity and acidity, and corrosion of, or formation of deposits on, metal surfaces. Excessive increase in viscosity can lead to a restricted flow of lubricant to the engine bearings resulting in inadequate lubrication on starting and/or inadequate cooling during engine running. Deterioration of engine component condition by excessive corrosion or deposition can lead to malfunctioning of the moving parts, and excessive formation of oil-insoluble materials can cause inadequate lubrication due to blockage of oil-ways. It is therefore very desirable that a lubricant of this type should show no more than a slight tendency to increase in viscosity and acidity during service.

The performance of a lubricant in these respects is frequently assessed by submitting it to an accelerated oxidation/corrosion test in which a sample of oil is maintained at a high temperature in contact with metal test pieces while a stream of air is bubbled through it for a prolonged period of time. Forms of this test are quoted in some Government and Engine Manufacturers' specifications for aero gas turbine lubricants. In one form of this test, used to assess oils for high temperature applications, the sample size is 90 grams, a temperature of  $400^{\circ}\text{F}$  ( $204^{\circ}\text{C}$ ), an air flow rate of 5 litres/hour and a test period of 72 hours are adopted as the test conditions, and one inch square plates of magnesium alloy, aluminium alloy, copper, silver and steel are used as the metal test pieces. A variation of this procedure uses a temperature of  $425^{\circ}\text{F}$  ( $218^{\circ}\text{C}$ ) and a test period of 48 hours. In these forms of the test, oils having poor resistance to oxidation at high temperatures give high viscosity and acidity increase and tend to corrode certain of the metals, especially copper and magnesium.

Various antioxidants are known for alleviating the above problems but in producing a final lubricant blend it is important that the particular combination of base oil and additives used should be clean in use and not give rise to unacceptable levels of deposits on the engine components. The above-mentioned oxidation tests assess the cleanliness of an oil in this respect by measuring the amount of insoluble material formed.

An object of the present invention is to provide a high temperature antioxidant which is capable of imparting outstanding oxidation stability to lubricating

oils intended for the lubrication of modern aero gas turbine engines, and which is clean in use.

In U.S. Pat. application Ser. No. 164,946 filed July 21, 1971 there is disclosed a diamine of formula



10

wherein A is a benzene nucleus substituted in the para position with a tertiary alkyl group having 4 to 9 carbon atoms and B is A or an alpha or beta naphthyl group. A process for the preparation of such a diamine is also 15 disclosed. There is provided in the aforementioned application Ser. No. 164,946 a process for the production of a diamine of Formula I.



which process comprises thermally rearranging a hydrazine of Formula II

30



40

wherein X is a benzene nucleus substituted in the para position with a tertiary alkyl group having 4 to 9 carbon atoms and Y is X or an alpha or beta naphthyl group.

By way of example, preparation of N,N,N'-tris-(4-t-octylphenyl)-4-octyl-1,2-phenylene diamine, subsequently referred to as "the diamine" is as follows:

394 g (1 mole) of 4,4'-diocetylphenyl amine were dissolved in 4 litres of acetone in a 5 litre beaker.

158 g (1 mole) of crystalline potassium permanganate were dissolved in 400 mls of distilled water at  $80^{\circ}\text{C}$  and added over the course of an hour to the amine solution, the mixture being heated to  $50^{\circ}\text{C}$  and stirred continuously. During the addition, manganese dioxide and N,N'-tetra-tris(-4-octylphenyl) hydrazine were precipitated. The complete mixture was stirred for a further 60 mins, after which time the precipitate was filtered off through a Buchner funnel and washed once with the filtrate. When the residue in the funnel was dry it was dissolved in 2 litres of toluene and the inorganic insolubles filtered from the solution. The toluene was then distilled under vacuum at  $80^{\circ}\text{C}$  in a rotary evaporation to give the solid hydrazine.

The powdered hydrazine was melted and maintained at  $106^{\circ}\text{C}$  for 20 hours. Upon cooling, the solid antioxidant was ground to a yellow crystalline solid.

65 Analysis of the solid antioxidant by thin layer chromatography revealed that it consisted of a mixture of monamine (15%), diamine (70%) and triamine (15%).

The diamine may be separated from the monoamine and triamine, e.g. by crystallisation, or the amines may be used admixed, in which case the antioxidant requires no further treatment.

These diamines are efficient antioxidants for lubricating compositions.

We have now discovered that antioxidant compositions of improved activity can be prepared by mixing such diamines with alkali metal derivatives of certain amines.

Thus according to the present invention there is provided an antioxidant composition comprising

a. a diamine of formula



and (b) an alkali metal derivative of an amine of formula



where x and y are as previously defined and n is 0, 1 or 2.

According to one preferred feature the amine of Formula II is of Formula



i.e., n is 0, and the alkali metal derivative is prepared by reacting the alkali metal with the amine.

According to another preferred feature, the amine of Formula II is again of Formula



and the alkali metal derivative in this case is prepared by reacting the alkali metal hydride with the amine.

According to yet another preferred feature the amine of Formula II is a diamine of Formula



i.e., n is 1. The alkali metal derivative may be prepared by reacting the diamine with an alkali metal or alkali metal hydride.

Suitable diamines of Formula I may be prepared by the method disclosed in Ser. No. 164,946 from 4,4'-di-t-butyl diphenylamine, (DODPA) 4,4'-di-t-hexyl diphenylamine; N [4-t-butyl-phenyl]- $\alpha$ -naphthylamine; N [4-t-octyl-phenyl]- $\alpha$ -naphthylamine; N[4-t-butyl-

phenyl]- $\beta$ -naphthylamine; N[4-t-octyl phenyl]- $\beta$ -naphthylamine, and, preferably, 4,4'-di-t-octyl diphenylamine.

The preferred diamine is N, N, N' - tris -(4-t-octylphenyl)-4-t-octyl-1,2-phenylene diamine (di-DODPA).

Diamines prepared by this method may have small amounts of monoamines and triamines associated with them.

10 Suitable amines of Formula II are those listed previously as suitable for conversion to diamines and also the diamines and triamines resulting from such conversions.

The alkali metal derivatives of the amine of Formula II may be prepared by reacting the alkali metal or metal hydride with an excess of the amine at a temperature in the range 150° to 200°C.

The preferred alkali metals are potassium and sodium.

20 The invention also includes a lubrication composition comprising a lubricating base oil, which may be mineral or synthetic, and up to 10% by weight of an antioxidant composition as described above.

The lubricating composition suitably contains between 0.01 and 6% by weight of the diamine, preferably between 2 and 4%. The lubricating composition suitably contains between 0.01 and 0.5% by weight of the alkali metal derivative, preferably between 0.04% and 0.2%.

30 The effect of the antioxidant composition is shown to maximum advantage by using it in a thermally stable liquid neutral polyester basestock. Such polyesters are prepared by reacting together under esterification conditions and in one or more stages:

35 i. an aliphatic mono- and/or polyhydric alcohol having 5-15, preferably 5-10, carbon atoms per molecule and having no hydrogen atoms attached to any carbon atom in a 2 position with respect to any -OH group and

ii. an aliphatic mono- and/or polycarboxylic acid having 2-14, preferably, 3-12 carbon atoms per molecule.

40 By 'polyester' is meant an ester having at least two ester linkages per molecule; it therefore includes diesters such as neopentyl glycol dipelargonate and di(2:2:4-trimethylpentyl) sebacate. The term neutral is used to mean a fully esterified product.

45 It is to be understood that in the esterification reaction described above there may be used more than one of any of the reactants mentioned e.g. a mixture of monocarboxylic acids and, in any case, the neutral ester product of the esterification reaction will sometimes consist of a mixture of different ester molecules, so the expression polyester is to be construed in this light.

50 Examples of suitable acids and alcohols that may be used in the preparation of the polyester are caprylic acid, capric acid, caproic acid, enanthic acid, pelargonic acid, valeric acid, pivalic acid, propionic acid, azelaic acid, 2:2:4-trimethylpentanol, neopentyl alcohol, neopentyl glycol, trimethylethylene, trimethylolpropane, pentaerythritol and dipentaerythritol.

55 Suitable polyesters are in the esters of trimethylolpropane, trimethylethylene, pentaerythritol and/or dipentaerythritol with one or more monocarboxylic acids having 3 to 10 carbon atoms, particularly one or more of those mentioned in the previous paragraph.

Most suitably, the trimethylolpropane and dicarboxylic acid are reacted in the molar ratio of 1:0.05/-0.75, preferably 1:0.075 - 0.4, the amount of monocarboxylic acid being sufficient to provide a carboxyl/hydroxyl balance in the reactants.

The invention is illustrated by the following examples

#### EXAMPLE 1

A potassium derivative of 4,4'-di-t-octyl diphenylamine (DODPA) was prepared by reacting 2g potassium with 100g of the amine at 190°C.

Two blends were then prepared using a synthetic ester basestock and subjected to the Rolls Royce 1001 oxidation test.

Air saturated with water vapour was bubbled at the rate of 250 ml/min through 50 ml samples of the blends at elevated temperature for 192 hours.

Deterioration of the samples because of oxidation were then measured in terms of fluid loss, acidity and viscosity change, and toluene insoluble materials after topping up the tested samples to their original volume with fresh material. The following results were obtained.

| Blend                                                      | Test Temp. °C | % Δ KV at 210°F | Δ TAN mg KOH/g | % Fluid Loss | % Toluene Insols |
|------------------------------------------------------------|---------------|-----------------|----------------|--------------|------------------|
| Ester Basestock + 4% by wt. diamine + 0.04% K DODPA        | 225           | 26.8            | 0.25           | 51           | <0.05            |
| Ester basestock + 4% by wt. diamine + 0.04% by wt. K DODPA | 230           | 45.0            | 0.1            | 60           | <0.05            |

Further samples of the blends were subjected to the Pratt and Whitney oxidation test.

A 90g. sample of each blend was taken and in it were

The cleanliness of the compositions was further assessed by the Roxana Panel Ccaker Test in which a sample of the blend containing diamine (di - DODPA) + K DODPA was splashed on to a weighed aluminium panel heated at 600°F for 8 hours and the nature and weight of the deposit on the panel were noted.

The following results were obtained:

| 10 | Panel           |               | Panel Description                  |  |
|----|-----------------|---------------|------------------------------------|--|
|    | Deposit Mg. 4.0 | % Coverage 50 | Type of deposit Sticky pale yellow |  |

The ester basestock was a complex ester prepared by esterifying caprylic acid, 1,1,1-trimethylol propane and sebacic acid in the molar ratio of 28:10:1. Diamine (di-DODPA) = N,N,N'-tris-(4t-octylphenyl)-4t-octyl-1,2-phenylene diamine. K DODPA = potassium derivative of 4,4'-di-t-octyl diphenylamine.

#### EXAMPLE 2

200g of 4,4'-di-t-octyl diphenylamine (DODPA) were melted in a round bottomed flask at about 100°C and the flask was flushed out with nitrogen gas. 6g of sodium hydride (ie. 12g of a 50% oil dispersion of sodium hydride) were added gradually to the stirred diphenylamine over a period of two hours. The reaction was vigorous and the contents of the flask turned dark green in colour. The product was heated and stirred for a further 2 hours after all the sodium hydride had been added. Upon cooling the product set to a green solid which consists of a mixture of sodium dioctyl diphenylamide and dioctyl diphenylamine. The alkali metal synergist was ready for use without any further treatment.

Two blends were then prepared using a synthetic ester basestock and subjected to the Rolls Royce 1001 oxidation test.

The following results were obtained:

| Additive Package                              | Temp. °C | % Fluid Loss | % Δ KV at 210°F | Δ TAN mg KOH/g | % toluene insol.       |
|-----------------------------------------------|----------|--------------|-----------------|----------------|------------------------|
| 4% diamine                                    | 230      |              |                 |                | Gelled after 100 hours |
| 4% diamine + 0.04% NaH/DODPA reaction product | 230      | 66.0         | 160.4           | 2.6            | Nil                    |

diamine (di-DODPA) = N,N,N'-tris-(4t-octylphenyl)-4t-octyl-1,2-phenylene diamine  
DODPA = 4,4'-di-t-octyl diphenylamine

placed one inch square plates of magnesium alloy, aluminium alloy, copper, silver and steel as test pieces. Dry air at a flow rate of 5 litres/hours was passed through the samples at 425°F for 48 hours. The viscosity and acidity increases of the samples, the sludges formed, the fluid losses and the corrosion of the metal plates were then determined.

The following results were obtained:

50 The ester basestock was a complex ester prepared by esterifying caprylic acid; 1,1,1-trimethylol propane and sebacic acid in the molar ratio of 28:10:1.

A potassium synergist was prepared by melting 30g. N,N,N'-tris(4t-octylphenyl)-4t-octyl-1,2-phenylene diamine under nitrogen in a flask. 0.4g metallic potassium was added and heating continued for 3 hours. The reaction product was then cooled and comminuted.

| Blend                                                      | % Δ KV at 100°F | Δ TAN mg KOH/g | Sludge mg | % Fluid Loss | Metal Weight Change |     |       |       |       |
|------------------------------------------------------------|-----------------|----------------|-----------|--------------|---------------------|-----|-------|-------|-------|
|                                                            |                 |                |           |              | Mg                  | Al  | Cu    | Ag    | Fe    |
| Ester basestock + 4% by wt. diamine                        | 16.8            | 1.1            | Nil       | 2.4          | Nil                 | Nil | -0.06 | -0.02 | -0.04 |
| Ester basestock + 4% by wt. diamine + 0.04% by wt. K DODPA | 16.2            | 3.5            | 5.3       | 1.9          | Nil                 | Nil | -0.05 | +0.06 | +0.06 |

A sodium synergist was prepared by reacting 16.3g of the diamine with 1g of a 50% oil dispersion of sodium hydride in hexane. After 2 hours refluxing the hexane solution was filtered to remove excess sodium hydride. The hexane was then stripped and the synergist cooled and comminuted. 5

Various blends were then prepared using synthetic ester basestocks and subjected to the Rolls Royce 1001 oxidation test.

The following results were obtained:

10

(I) and

| Example | Additive Package                 | Basestock | Temp °C | % Fluid Loss | % Δ kv at 210°F | Δ Tan mg KOH/g             | % Toluene Insolubles |
|---------|----------------------------------|-----------|---------|--------------|-----------------|----------------------------|----------------------|
| 3       | 4% diamine                       | Ester A   | 225     |              |                 |                            |                      |
| 4       | 4% diamine + 0.04% K diamine     | Ester A   | 230     | 64.2         | 50              | Gelled after 100 hours 1.4 | Nil                  |
| 5       | 4% diamine + 0.04% K diamine     | Ester A   | 235     | 78.8         |                 | Gelled after 190 hours     |                      |
| 6       | 6% diamine + 0.06% K diamine     | Ester A   | 230     | 55           | 40.4            | 0.7                        | Nil                  |
| 7       | 6% diamine + 0.06 K diamine      | Ester A   | 235     | 77.2         | 103.6           | 1.65                       | Nil                  |
| 8       | 4% diamine                       | Ester B   | 225     |              |                 |                            |                      |
| 9       | 6% diamine + 0.06% K diamine     | Ester B   | 230     | 62.6         | 34.8            | Gelled after 100 hours 0.3 | Nil                  |
| 10      | 6% diamine + 0.06% K diamine     | Ester B   | 235     | 77.2         | 50.7            | 0.55                       | Nil                  |
| 11      | 4% diamine + 0.04% Na derivative | Ester A   | 230     | 71.4         | 190             | 2.75                       | Nil                  |

diamine (di-DODPA = N,N,N',N'-tris(4-t-octylphenyl)-4-t-octyl-1,2-phenylene diamine  
K diamine = potassium derivative of the diamine  
Na diamine = sodium derivative of the diamine

Ester A was a complex ester prepared by esterifying 30 caprylic acid, 1,1,1-trimethylol propane and sebacic acid in the molar ratio of 28:10:1.

Ester B was prepared by esterifying monopentaerythritol with a mixture of normal alkanoic acids of chain length C<sub>4-10</sub> having an average chain length of C<sub>7</sub>. 35

Further blends were subjected to the Pratt and Whitney oxidation test.

The following results were obtained.



8

b. an alkali metal amide of an amine of the formula



(II)

| Example | Additive Package                           | Basestock | % Fluid Loss | % Δ kv at 100°F | Δ TAN mg KOH/g | Sludge mg | Metal Weight Change |       |       |       |       |
|---------|--------------------------------------------|-----------|--------------|-----------------|----------------|-----------|---------------------|-------|-------|-------|-------|
|         |                                            |           |              |                 |                |           | Mg                  | Al    | Cu    | Ag    | Fe    |
| 12      | 3% DODPA + 0.5% OPANA                      | Ester A   | 2.3          | 31.2            | 5.0            | 1.9       | -0.02               | +0.02 | +0.01 | +0.03 | +0.03 |
| 13      | 4% diamine + 0.04% K diamine + 0.3% PL 297 | Ester A   | 3.2          | 12.3            | 0.5            | 7.9       | -0.01               | -0.01 | -0.13 | -0.02 | -0.01 |
| 14      | 4% diamine + 0.04% K diamine + 0.3% PL 297 | Ester B   | 2.1          | 12.5            | 0.6            | 3.1       | -0.01               | -0.03 | -0.13 | -0.02 | +0.07 |

PL 297 = a salt of salicylaminoguanidine and one or more C<sub>10-18</sub> fatty acids  
DODPA = 4,4'-diocylidiphenylamine  
OPANA = 4-octylphenyl- $\alpha$ -naphthylamine

Examples 3, 8 and 12 are provided for comparative purposes only, Example 10 being an example of a very good prior art additive combination. 55

Examples 4 - 7, 9 - 11 and 13 and 14 clearly illustrate the enhanced antioxidant activity of combinations of N,N,N'-tris(4-t-octylphenyl)-4-t-octyl-1,2-phenylene diamine and its potassium or sodium derivative when compared with the diamine itself or a prior art combination.

We claim:

1. An antioxidant composition comprising  
a. a diamine of the formula

where X is a benzene nucleus substituted in the para position to the nitrogen atom with a tertiary alkyl group having 4 to 9 carbon atoms and Y is selected from the group consisting of a benzene nucleus substituted in the para position with a tertiary alkyl group having 4 to 9 carbon atoms, an alpha naphthyl group and a beta naphthyl group, and n is 0, 1, or 2, the weight ratio of the diamine of Formula I to the alkali metal amide being 1:1 to 12:1.

2. An antioxidant composition according to claim 1, 65 wherein n is 0 and the alkali metal amide is prepared by reacting an alkali metal with the amine of Formula

II in the presence of an excess of said amine at a temperature in the range of 150° to 200°C.

3. An antioxidant composition according to claim 1 wherein  $n$  is 0 and said alkali metal amide is prepared by reacting an alkali metal hydride with an excess of the amine of Formula II at a temperature in the range 150° to 200°C.

4. An antioxidant composition according to claim 1 where  $n$  is 1.

5. A lubricating composition comprising a lubricating base oil and up to 10% by weight of an antioxidant composition according to claim 1.

6. A lubricating composition according to claim 5 wherein the diamine of Formula I is present in an amount in the range 0.01 to 6% by weight.

7. A lubricating composition according to claim 6 wherein the diamine is present in an amount in the range 2 to 4% by weight.

8. A lubricating composition according to claim 5 wherein the alkali metal amide is present in an amount in the range 0.01 to 0.5% weight.

9. A lubricating composition according to claim 8 wherein the alkali metal amide is present in an amount in the range 0.04 to 0.2% by weight.

10. A lubricating composition comprising a synthetic 25

polyester base oil and up to 10% by weight of an antioxidant composition according to claim 1.

11. An antioxidant according to claim 1, wherein the diamine is N,N,N'-tris-(4-t-octylphenyl)-4-t-octyl-1,2-5 phenylene diamine.

12. An antioxidant according to claim 2, wherein the amine of Formula II is 4,4'-di-t-butyl-diphenylamine; 4,4'-di-t-hexyl-diphenylamine; N [4-t-butylphenyl]- $\alpha$ -naphthylamine; N [4-t-octylphenyl]- $\alpha$ -naphthylamine; 10 N [4-t-butylphenyl]- $\beta$ -naphthylamine; N [4-t-octylphenyl]- $\beta$ -naphthylamine or 4,4'-di-t-octyl-diphenylamine.

13. An antioxidant composition according to claim 4, wherein the amine of Formula II is N,N,N'-tris-(4-t-octyl-1,2-phenylene diamine.

14. An antioxidant composition in accordance with claim 1, wherein the diamine of Formula I is a diamine obtained from a thermal conversion of an amine selected from the group consisting of 4,4'-di-t-butyl-20 diphenylamine; 4,4'-di-t-hexyl-diphenylamine; N[4-t-butylphenyl]- $\alpha$ -naphthylamine; N[4-t-octylphenyl]- $\alpha$ -naphthylamine; N[4-t-butylphenyl]- $\beta$ -naphthylamine; N[4-t-octylphenyl]- $\beta$ -naphthylamine and 4,4'-di-t-octyl-diphenylamine.

\* \* \* \* \*

30

35

40

45

50

55

60

65